

# UNITED STATES PATENT OFFICE.

JAMES ELIOT BOOGIE, OF WILMINGTON, DELAWARE, ASSIGNOR TO E. I. DU PONT DE NEMOURS & COMPANY, OF WILMINGTON, DELAWARE, A CORPORATION OF DELAWARE.

## NONCRACKING COATING COMPOSITION AND ARTIFICIAL LEATHER MADE THEREWITH.

1,412,770.

Specification of Letters Patent. Patented Apr. 11, 1922.

Application filed June 13, 1918. Serial No. 239,903.

To all whom it may concern:

Be it known that I, JAMES ELIOT BOOGIE, of Wilmington, in the county of New Castle and in the State of Delaware, have invented 5 a certain new and useful Improvement in Noncracking Coating Compositions and Artificial Leather Made Therewith, and do hereby declare that the following is a full, clear, and exact description thereof.

10 My invention relates particularly to coating compositions and artificial leather made therewith, in which oils are used which could not previously be used with advantage, owing to the tendency thereof to make 15 the coated product crack under the influence of comparatively low temperatures.

The object of my invention is to provide 20 coating compositions and artificial leather made therewith, in which oils are used which could not previously be used with advantage because of their low fluidity or great viscosity at the lower atmospheric temperatures. The previously treated oils, that is to say oils which have been blown, 25 or oxidized by exposure to the air or oxygen, or polymerized, could not be used with advantage in coating compositions utilized in the making of artificial leather, as the use of such oils would almost invariably make the coated product crack when 30 subjected to a temperature of 0° C. or lower and sharply bent or creased. This property rendered the use of artificial leather made with oils of this character 35 unsuitable for outdoor purposes, as for example in automobile upholstering. I have discovered that this is due to the low fluidity or great viscosity of such oils at these temperatures.

40 The object of my invention is, therefore, to utilize oils of this character by adding to the compositions containing the same constituents to increase their fluidity.

A further object is to add to such compositions non-volatile solvents having a great degree of fluidity at the lower temperatures to accomplish this end.

45 Another object of my invention is to add to compositions of this character esters of the lower alcohols, such for example as methyl or ethyl alcohol with the higher fatty acids, such as lauric, myristic and palmitic acids or oleic and ricinoleic acid.

Further objects of my invention will ap-

pear from the detailed description thereof 55 contained hereinafter.

While my invention is capable of embodiment in many different forms, for the purpose of illustration I shall describe only certain forms thereof hereinafter.

60 For example in carrying out my invention, I may proceed as follows:

Cloth, split leather or other material may be coated in any suitable manner with one or more coats of a composition made in the following way: The composition may be comprised of one part by weight nitrocellulose, two parts by weight of blown rape seed or cottonseed oil, one part by weight of a non-volatile solvent having a high 70 degree of fluidity at low temperatures such for example as the methyl or ethyl esters of the mixed fatty acids from cocoanut oil and about seven parts by weight of volatile solvents comprising 5 parts by weight of 75 ethyl acetate, and 3 parts by weight of benzene. It will be understood, however, that for the non-volatile solvents I may use any material having the properties herein referred to, and for example I may use 80 for this purpose any of the esters of the lower alcohols with the higher fatty acids, but I prefer to use one or more of the esters of methyl or ethyl alcohol with the saturated fatty acids, such for example as lauric, 85 myristic and palmitic acids, although the corresponding esters of unsaturated acids, such as oleic or ricinoleic acid may be used.

Again the esters may be the corresponding esters of the mixed fatty acids from castor oil or of the mixed fatty acids of cottonseed oil. By referring to such substances as non-volatile solvents I merely mean to state, however, that as to their solvent power they need only have the property of dissolving in the oil used in the composition, and of mixing with the nitrocellulose and volatile solvents present in the composition. Furthermore, it is desirable that these non-volatile solvents be of such a character that 100 under the influence of the lower atmospheric temperatures they will not crystallize out in the coating to produce a white "bloom". Furthermore, it will be understood that the quantity of nitrocellulose 105 and volatile solvents present in the composition is such as to form a nitrocellulose jelly which is mixed with the other constit-

uents, and then applied to the fabric to be coated.

While I have described my invention above in detail, I wish it to be understood that many changes may be made therein without departing from the spirit thereof. Also, although in certain of the claims I have merely used the term "blown oil" instead of the term "blown or polymerized oil", it is to be understood that the term "blown oil" has been adopted for brevity, and not to exclude polymerized oil; since by virtue of the present invention not only blown oil but also polymerized oil can be used in the coating and yet cold cracking of the coating be avoided, so that, from this point of view the oils are equivalents.

I claim:

1. A composition comprising a nitrocellulose, a blown oil and a non-volatile solvent imparting flexibility in the cold and adapted to prevent cold-cracking of the composition when in the form of a coating.

2. A composition comprising a nitrocellulose, blown cottonseed oil and a non-volatile solvent adapted to prevent cold-cracking of the composition when in the form of a coating.

3. A composition comprising a nitrocellulose, a blown oil and a non-volatile solvent containing an ester of a lower alcohol with a higher fatty acid adapted to prevent cold-cracking of the composition when in the form of a coating.

4. A composition comprising a nitrocellulose, blown cottonseed oil and a non-volatile solvent containing an ester of a lower alcohol with a higher fatty acid adapted to prevent cold-cracking of the composition when in the form of a coating.

5. A composition comprising a nitrocellulose, a blow oil and a non-volatile solvent containing esters of a lower alcohol with the mixed fatty acids of cocoanut oil adapted to prevent cold-cracking of the composition when in the form of a coating.

6. A composition comprising a nitrocellulose, blown cottonseed oil and a non-volatile solvent containing esters lower alcohol with the mixed fatty acids of cocoanut oil adapted to prevent cold-cracking of the composition when in the form of a coating. 50

7. A coating composition comprising a nitrocellulose jelly, a blown oil and a non-volatile solvent imparting flexibility in the cold and adapted to prevent cold-cracking of the coating. 55

8. A coating composition comprising a nitrocellulose jelly, blown cottonseed oil and a non-volatile solvent adapted to prevent cold-cracking of the coating. 60

9. A coating composition comprising a nitrocellulose jelly, a blown oil and a non-volatile solvent containing an ester of a lower alcohol with a higher fatty acid 65 adapted to prevent cold-cracking of the coating.

10. A coating composition comprising a nitrocellulose jelly, blown cottonseed oil and a non-volatile solvent containing an ester of a lower alcohol with a higher fatty acid 70 adapted to prevent cold-cracking of the coating.

11. A coating composition comprising a nitrocellulose jelly, a blown oil and a non-volatile solvent containing esters a lower alcohol with the mixed fatty acid of cocoanut oil adapted to prevent cold-cracking of the coating. 75

12. A coating composition comprising a nitrocellulose jelly, blown cottonseed oil and a non-volatile solvent containing esters of a lower alcohol with the mixed fatty acids of cocoanut oil adapted to prevent cold-cracking of the coating. 80 85

In testimony that I claim the foregoing I have hereunto set my hand.

JAMES ELIOT BOOGE.

Witnesses:

G. D. HOPKINS,  
STANLEY L. ABRAMS.